

## UNITED STATES PATENT OFFICE

2,069,774

DELUSTERED CELLULOSIC STRUCTURE AND  
METHOD FOR PREPARING SAME

Ebenezer Emmet Reid, Baltimore, Md., assignor,  
by mesne assignments, to E. I. du Pont de  
Nemours & Company, Wilmington, Del., a cor-  
poration of Delaware

No Drawing. Application September 15, 1934,  
Serial No. 744,267

11 Claims. (Cl. 106—40)

This invention relates to cellulosic structures such as filaments, threads, fabrics, sheets, films, caps, tubing, or the like. More particularly, this invention relates to cellulosic structures of the type just mentioned having a subdued or low luster and/or that are more or less opaque.

In the ordinary methods of preparing cellulosic structures, such as filaments, threads, films, caps, tubing, etc., from viscose, cuprammonium, nitro-cellulose, cellulose acetate and other cellulosic solutions (without the addition of opaques and/or low luster-inducing agents to the solutions), the products are transparent or translucent and/or very highly lustrous. For many purposes, transparency, brilliant sheen and luster are not desirable and thus restrict the uses of the materials. Recently, various methods have been proposed for producing cellulosic structures having a low or subdued luster and/or opacity.

I have found that I can produce cellulosic structures characterized by a low luster and/or opacity by incorporating therein a sulfone or sulfoxide of the character described in detail hereinafter which imparts opacity and/or low luster by remaining in the cellulosic structure.

An object of the invention comprises the production of new opacified and/or low luster cellulosic structures. A further object of the invention relates to the production of novel cellulosic structures containing organic compounds which remain in the finished article and which impart opacity and/or low luster. Other objects of the invention will appear hereinafter.

The objects of the invention are accomplished in general by incorporating in the cellulosic solution from which the structure is to be produced an opaque and/or a low luster-inducing agent of the type hereinafter more fully explained.

So far as the instant invention is concerned, each closed chain or carbon or hetero- atom or combination of carbon and hetero- atoms will be considered a nucleus. Thus, benzene, naphthalene and carbazole have one, two, and three nuclei respectively.

These opaques and/or low luster-inducing agents, which are preferably white in color, possess a sufficiently low vapor pressure and are sufficiently inert to resist the change or removal from the cellulosic structure in the ordinary process of making and finishing the same during the manufacture thereof. They also effectively resist removal or change during any of the usual processes to which the finished cellulosic structure may be subjected, such as boiling-off, dyeing, bleaching, washing, ironing, etc. These substances are incompatible with the mass of the substance constituting the final product. They may be soluble but, in the preferred embodiment of this invention, they are insoluble in the solution from which the structure is prepared.

Highly effective delusterants function in particular by reason of their opacifying power which is a function of the difference in refractive index between the delusterant particle and the surrounding medium. Those in my preferred range differ from the index of the medium by at least 0.10 and the greater this difference, the more effective the compound as an opacifier and/or delusterant. Most organic compounds have several indexes and the statement just made refers to the highest index of the compound or to any one of the several indexes.

As illustrative examples of sulfones coming within the scope of this invention are the following:

Dibenzyl ether of *p,p'* dihydroxy diphenyl sulfone



Dinaphthyl ether of diphenylol sulfone



Difurfuryl sulfone



The low luster-inducing and/or opaque agent contemplated by this invention is an organic sulfone or sulfoxide having at least one and preferably two or more carboxylic or heterocyclic nuclei highly deficient in hydrogen, and their colorless derivatives such as those formed by substituting the following groups for hydrogen: —R, —O—R, —S—R, —Se—R, —Te—R, —NH—R, —CO—R, hydroxy alkyl or halogen, in which "R" may be an alkyl, aryl, alkaryl, aralkyl, or a heterocyclic group.

## 2,7 dibenzenesulfonyl carbazole

5



10

## 3-benzene sulfonyl phthalimide

15



15

## s-Dibenzthiazyl sulfonyl ethane

20



25

Dinaphthyl sulfone resin  
Refractive index—1.70

30



35

## Alphanaphthyl phenyl sulfone

40



45

## Beta-naphthyl tolyl sulfone

50



55

## Phenyl p-chlorophenyl sulfone

60



65

## Beta-naphthyl p-chlorophenyl sulfone

70

## Diphenyl sulfone dichlorodiethyl ether resin

75



75

## 1,3,5 trinaphthyl trisulfonyl benzene

5



10

## 1,3,5 triphenyl trisulfonyl benzene

15



20



25



30



35



40

Di-alpha-naphthyl sulfone  
Refractive index—1.66; 1.73; 1.79

45



50



55



60



65



70

5 p-p' Dichlorodiphenyl sulfone  
Refractive index—1.53; 1.75



10 Methyl-beta-naphthyl sulfone



15 As examples of sulfoxides may be mentioned  
15 the above sulfones in which the SO<sub>2</sub> group is re-  
placed by an SO group.

20 Other specific sulfones which may be men-  
tioned as included within the broad scope of  
this invention are:

20 Trimethylene trisulfone (ref. index—1.60; 1.66)  
Hexamethyl trimethylene trisulfone, and

25 The sulfones and sulfoxides derived from spi-  
ro-bis-thiocyclobutane [see Rec. Trav. Chim.  
52-499, (1933)]

25 The organic compounds contemplated as de-  
lusterants in accordance with the principles of  
this invention are embraced in the following  
formulae:



and



35 in which R or R<sub>1</sub> may be any organic group  
having a carbon atom which is directly linked  
to the sulfur atom.

40 The scope of this invention is not intended to  
include sulfonic acids or salts of sulfonic acids  
except as set forth by the above type formulae.

45 Organic compounds of the character described  
which have relatively high indexes of refraction  
and which are preferred on the basis of cost,  
color stability, acid insolubility and effectiveness  
are the following:

50 Methyl-beta-naphthyl sulfone,  
Di-alpha-naphthyl sulfone,  
1,3,5 Trinaphthalene-sulfonyl benzene,  
1,3,5 Tribenzene-sulfonyl benzene,  
1,2 Di-naphthyl ethylene disulfone,  
Triphenylmethylene trisulfone,  
Methyl dinaphtho sulfone.

55 The quantity of the low luster-inducing  
and/or opaques agent which may be used may  
vary within wide limits, depending principally  
upon the opaques and luster desired in the final  
product. Cellulosic structures containing these  
low luster-inducing and/or opaques agents in  
60 amounts ranging from 0.10-20.0% by weight have  
given satisfactory results, but, of course, it is  
obvious that smaller or larger quantities may be  
employed as desired. When a viscose solution is  
employed, satisfactory results may be secured if  
65 it contains 7% cellulose and from 0.01-1.5% more  
or less of the low luster-inducing and/or opaques  
agent.

70 If desired, the low luster-inducing agents con-  
templated by the instant invention may be used  
in combination with each other and/or with  
other low luster-inducing agents, such as mineral  
oil, petroleum jelly, waxes, paraffin, benzene,  
toluene, pine oil or inorganic pigments, such as  
titanium oxide, lithopone, zinc sulfide, etc.

75 The low luster-inducing agent may be added to

the solution at any stage in the course of the  
manufacture thereof, or after the preparation of  
the solution and prior to the spinning, extrusion  
or casting operation. It may be added directly,  
if the particle size is satisfactory, or after suit-  
able adjustment of the particle size by any of the  
well known methods, such as emulsification,  
grinding in a colloid mill or pebble mill, or in the  
form of a suspension or emulsion prepared with  
or without the assistance of suitable dispersing  
agents or protective colloids, such as soaps, sul-  
fonated oils, alkyl naphthalene sulfonates, sodium  
caseinate, etc., or combinations thereof.

10 In order to more fully explain the principles  
of this invention, the following illustrative ex-  
amples are given.

15 Example I.—A sample of beta-naphthyl phenyl  
sulfone (melting point 115°) is emulsified  
preferably in the manner described in the co-  
pending application of W. W. Heckert, filed Octo-  
ber 11, 1934 as Serial No. 747,933, Example I. The  
20 resulting emulsion is used in making up  
viscose in such proportions that the final viscose  
contains 7% cellulose and 0.4% beta-naphthyl  
phenyl sulfone. The viscose is spun into rayon or  
25 cast into films in the usual manner. The products  
are characterized by a desirable opacity and  
low luster.

30 Example II.—Four hundred parts of di-alpha-  
naphthyl sulfone (melting point 188°) are ground  
with 600 parts of water, 8 parts of sodium  
caseinate, and 4000 parts of pebbles in a pebble  
mill until all the particles are reduced to a par-  
ticle size of 4 microns or less in diameter. The  
35 resulting dispersion is used in making up viscose  
in such proportions that the viscose contains 7%  
cellulose and 0.4% di-alpha-naphthyl sulfone.  
The viscose is cast into films or spun into rayon.  
The products have a desirable opacity and low  
40 luster, much lower than that obtained with min-  
eral oil, resembling that obtained with inorganic  
pigments.

45 Example III.—A sample of di-alpha-naphthyl  
sulfoxide (melting point 162°) is ground in the  
manner described in Example II. The resulting  
dispersion is used in making up viscose in such  
proportions that the viscose contains 7% cellulose  
and 0.1% di-alpha-naphthyl sulfoxide. The vis-  
cose is spun into rayon or cast into film in the  
usual manner. The resulting products have a de-  
50 sirable opacity and moderately low luster.

55 Example IV.—Four hundred parts of a diphe-  
nyloxy sulfone-dichlorodiethyl ether resin are  
ground in the manner described in Example I.  
The resulting pigment slurry is filtered (with the  
aid of a flocculating agent if necessary), dried and  
then dispersed in 1,600 parts of acetone by any  
suitable means such as violent agitation, grind-  
ing or passage through a colloid mill. The re-  
sulting acetone dispersion is used in making up  
a cellulose acetate spinning solution in such pro-  
portions that there is present one part of the  
resin for each ten parts of cellulose acetate. The  
60 cellulose acetate solution is spun into filaments  
or cast as a film in the usual manner. The prod-  
ucts have a desirable opacity and low luster.

65 It is to be understood that these examples do  
not in any way restrict the invention thereto but  
merely illustrate several specific and preferred  
70 embodiments which have given satisfactory re-  
sults.

75 Though the preferred embodiments of this in-  
vention contemplate the incorporation of the low  
luster-inducing agent in the solution at some time

prior to the extrusion or casting thereof, satisfactory results may be secured also by applying the low luster-inducing agent to a previously formed cellulosic structure. In other words, the 5 low luster-inducing agent may be applied to the final cellulosic structure by an after-treatment.

Though the invention has been specifically described in connection with the viscose process, it 10 is obvious that the principles thereof are equally applicable to the cuprammonium cellulose, cellulose nitrate, and cellulose acetate processes.

In the case of cellulosic solutions of wholly organic solvents, it is only necessary that a suitable choice of sulfone or sulfoxide be made so 15 that the solubility characteristics do not interfere. It has already been pointed out that the low luster-inducing substance must be incompatible with the mass of substance constituting the final product. In addition, in the case of 20 cellulose acetate or nitrate spinning solutions, it is preferable that the low luster-inducing substance be insoluble in the solvent employed. However, resinous materials and certain crystallized substances, soluble in the solvent, precipitate on 25 the evaporation of the solvent) in the cellulose acetate in the form of fine amorphous or crystalline particles sufficiently small and well distributed to avoid harmful effect on the physical properties of the resulting structure. The advantage 30 in such cases lies in avoiding the necessity for emulsifying or grinding the compounds to obtain suitable subdivision. Suitable compounds may be readily selected from any specific system by one skilled in the art.

35 While the invention has been described generally with respect to the use of the various compounds mentioned herein in opaquing cellulosic structures prepared by casting and/or spinning methods, it is desired to emphasize the fact that 40 these compounds are of special benefit in the spinning of artificial silk. Thus, undelustered artificial silk has a shade and luster which is undesired for a great many purposes. In accordance with the present invention, it is possible to 45 produce artificial silk, particularly of the regenerated cellulose type prepared from viscose or cuprammonium cellulose, having a pleasing dull appearance, the dullness being of any degree desired, in which the opaquing and/or delustering 50 agent is uniformly distributed and which does not interfere with the tenacity of the yarn to any large extent.

Since it is obvious that various changes and 55 modifications may be made in the above description without departing from the nature or spirit thereof, this invention is not restricted thereto except as set forth in the claims.

1. Artificial cellulosic filaments and pellicles 60 containing a cellulosic base and a finely divided, incompatible delustering and/or opaquing agent comprising an organic compound embraced by the formula:



65 in which R or R<sub>1</sub> may be any organic group having a carbon atom which is directly linked to the sulfur atom, and in which R<sub>2</sub> represents one or two oxygen atoms.

70 2. Artificial cellulosic filaments and pellicles 75 containing a cellulosic base and a finely divided, incompatible delustering and/or opaquing agent comprising an organic compound having two or more carbocyclic or heterocyclic nuclei highly

deficient in hydrogen and embraced by the formula;



and in which R or R<sub>1</sub> may be any organic group having a carbon atom which is directly linked to the sulfur atom, and in which R<sub>2</sub> represents one or two oxygen atoms.

3. Artificial cellulosic filaments and pellicles 1 containing a cellulosic base and a finely divided, incompatible delustering and/or opaquing agent comprising an organic compound embraced by the formula;



in which R or R<sub>1</sub> may be any organic group having a carbon atom which is directly linked to the sulfur atom, and in which R<sub>2</sub> represents one or two oxygen atoms, said compound having an index of refraction differing by at least 0.1 from the index of refraction of the cellulosic base.

4. Artificial cellulosic filaments and pellicles 2 containing a cellulosic base and a finely divided, incompatible delustering and/or opaquing agent comprising an organic compound having two or more carbocyclic or heterocyclic nuclei highly deficient in hydrogen and embraced by the formula;



and in which R or R<sub>1</sub> may be any organic group having a carbon atom which is directly linked to the sulfur atom, and in which R<sub>2</sub> represents one or two oxygen atoms, said compound having an index of refraction differing by at least 0.1 from the index of refraction of the cellulosic base.

5. Artificial cellulosic filaments and pellicles 4 containing a cellulosic base and 0.1% to 20% of a finely divided, incompatible, substantially white, delustering and/or opaquing agent comprising an organic compound having two or more carbocyclic or heterocyclic nuclei highly deficient 41 in hydrogen and embraced by the formula;



50 in which R or R<sub>1</sub> may be any organic group having a carbon atom which is directly linked to the sulfur atom, and in which R<sub>2</sub> represents one or two oxygen atoms.

6. Artificial cellulosic filaments and pellicles 55 containing a cellulosic base and 0.1% to 20% of a finely divided, incompatible, substantially white, delustering and/or opaquing agent comprising an organic compound having two or more carbocyclic or heterocyclic nuclei highly deficient 60 in hydrogen and embraced by the formula;



65 in which R or R<sub>1</sub> may be any organic group having a carbon atom which is directly linked to the sulfur atom, and in which R<sub>2</sub> represents one or two oxygen atoms, said compound having an index of refraction differing by at least 0.1 from the index of refraction of the cellulosic base.

7. Artificial cellulosic filaments and pellicles 70 containing a cellulosic base and 0.1% to 20% of a finely divided, incompatible, substantially white, delustering and/or opaquing agent com- 75

prising an organic compound embraced by the formula:



5 in which R or R<sub>1</sub> may be any organic group having a carbon atom which is directly linked to the sulfur atom, and in which R<sub>2</sub> represents one or two oxygen atoms, said compound having an 10 index of refraction differing by at least 0.1 from the index of refraction of the cellulosic base.

8. Artificial cellulosic filaments and pellicles containing a cellulosic base and a finely divided, incompatible delustering and/or opaquing agent 15 comprising an organic compound taken from the group consisting of methyl-beta-naphthyl sulfone, di-alpha-naphthyl sulfone, 1,3,5 trinaph-

thalene-sulfonyl benzene, 1,3,5 tribenzene-sulfonyl benzene, 1,2 di-naphthyl ethylene disulfone, triphenylmethylen trisulfone and methyl dinaphtho sulfone.

9. Artificial cellulosic filaments and pellicles 5 containing a cellulosic base and a finely divided, incompatible delustering and/or opaquing agent comprising methyl-beta-naphthyl sulfone.

10. Artificial cellulosic filaments and pellicles containing a cellulosic base and a finely divided, 10 incompatible delustering and/or opaquing agent comprising di-alpha-naphthyl sulfone.

11. Artificial cellulosic filaments and pellicles containing a cellulosic base and a finely divided, 15 incompatible delustering and/or opaquing agent comprising 1,3,5 triphenyl-trisulfonyl benzene.

EBENEZER EMMET REID.